

Oct. 10, 1950

2,524,895

F. G. DODGE  
PUCKERING A THERMOPLASTIC FABRIC  
BY HEATING ONE SIDE THEREOF  
Filed Oct. 31, 1945



INVENTOR.

FREDERICK G. DODGE.

BY

*I. Salter & A. Levinson*  
ATTORNEYS

## UNITED STATES PATENT OFFICE

2,524,895

PUCKERING A THERMOPLASTIC FABRIC BY  
HEATING ONE SIDE THEREOFFrederick G. Dodge, Cumberland, Md., assignor  
to Celanese Corporation of America, a corpora-  
tion of Delaware

Application October 31, 1945, Serial No. 625,745

11 Claims. (Cl. 8—131)

1

This invention relates to the production of novel decorative patterned fabrics, and relates more particularly to the production of novel patterned textile fabric webs comprising filamentary materials having a basis of a thermoplastic material.

An object of this invention is the production of novel textile fabrics having an attractive surface exhibiting a quilted effect and made of or containing yarns and filaments having a basis of a thermoplastic material.

Another object of this invention is to provide a rapid and economical process whereby said novel patterned fabrics may be produced in a continuous manner.

A further object of this invention is the provision of simple and inexpensive apparatus adapted for the production of said decorative fabrics.

Other objects of this invention will appear from the following detailed description and the accompanying drawing.

In the drawing,

Fig. 1 is a view in perspective of the apparatus employed in connection with my novel process showing a roll of fabric, a fabric heating element and the fabric feed and take-off means; and

Fig. 2 is a cross-sectional view of the novel fabric produced in accordance with my process.

Like reference numerals indicate like parts in both views of the drawing.

Fabrics made of or containing yarns and filaments having a basis of a thermoplastic textile material and presenting a three-dimensional patterned effect have heretofore been produced by embossing operations. In such embossing operations, the fabric is passed between heated rotating rolls, one of which carries the desired pattern in relief while the other carries the pattern in intaglio. The heated rolls are rotated in such a manner that the raised portions of one roll register with the depressions in the other and the combined action of heat and pressure serves to distort the thermoplastic material permanently and to yield a three-dimensional, patterned material. Any change in the pattern design requires a different set of engraved rolls which are quite costly. Furthermore, the pattern is constantly repeated in the embossed fabric at relatively short intervals, and therefore, a non-repetitive random pattern cannot be obtained.

I have now discovered that an unusually attractive random, three-dimensional pattern effect, i. e. a random, quilted effect, may be produced on fabrics made of or containing yarns or filaments having a basis of a thermoplastic material in a

rapid and economical manner. In accordance with my novel process, said patterned fabrics may be obtained by passing fabrics made of or containing yarns of a thermoplastic material, with no substantial tension thereon, over a surface heated to a temperature sufficiently high to effect a softening or slight melting of the thermoplastic materials contained in said fabrics. The softening or slight melting which takes place causes a localized shrinking or buckling of the fabric with the formation of an attractive, random overall pattern effect of a quilted appearance. The pattern formed is permanent and does not undergo any change during use.

The temperature at which the heated surface is maintained to produce the desired effect may vary. Where fabrics made of or containing yarns and filaments having a basis of cellulose acetate or other organic derivative of cellulose are employed, the temperature of the surface is most preferably held between 250 and 280° C. The fabric is fed at a rate of 1-to-2 yards a minute with the heated surface being of such dimensions that the fabric is in contact therewith for from 1 to 5 seconds.

In order further to illustrate my invention, reference may be had to the accompanying drawing wherein there is shown a simple and effective apparatus employed in the production of my novel patterned fabrics.

Referring now to the drawing and more particularly to Fig. 1, there is shown a roll of fabric, generally indicated by reference numeral 5, wound on a suitable support 6 carried on a centrally disposed shaft 7 adapted to fit into suitable bearings, such as roller bearings (not shown), to permit roll 5 to be freely rotatable and permit the fabric 8 to be readily unrolled therefrom. Roll 5 is rotated and fabric 8 thus paid off through the action of a positively driven, rubber-covered friction roll 9 which rests on the upper portion of said roll 5. Friction roll 9 is rotated by a belt and pulley arrangement, the pulley 10 being mounted on shaft 11, on which roll 9 is mounted, and held in position thereon by a set screw 12. Belt 13 circles pulley 10 and is driven in any suitable manner (not shown) to cause friction roll 9 to rotate in the direction shown. Shaft 11 passing through friction roll 9 may be supported in suitable bearings (not shown) adapted to allow the friction roll 9 to float which enables it to bear down on fabric roll 5 and to maintain the desired frictional contact therewith through the force of gravity.

The rotation of friction roll 9 causes the thermoplastic fabric 8 to be paid off fabric roll 5 and to come in contact with a heated metal plate 14 maintained at the desired temperature by any suitable heating means. For highly accurate control of the temperature, I preferably employ electrical resistance coils (not shown) suitably disposed beneath or within said plate. In lieu of a metal plate, a ceramic material or any other material capable of being heated to and maintained at the desired temperature may also be employed. Plate 14 may be supported in any convenient manner as on brackets 15, only one of which is shown.

When the fabric 8 comes into contact with heated plate 14, the elevated temperature at which said plate is maintained causes a softening and/or melting of the thermoplastic material. This softening action produces a non-uniform buckling of the fabric with the formation of an overall pattern effect. The pattern effect comprises a substantially continuous series of raised or puffed areas 16, as more clearly shown in Fig. 2, varying in size and shape, the narrow depressions between said raised areas being very slightly stiffened.

The fabric 8 after passing across plate 14 and having a pattern produced therein, is withdrawn by the action of a rotating take-off roll 17 driven by means of a belt 18, which is in frictional contact with a pulley 19 mounted on a shaft 20 passing through said take-off roll 17. Pulley 19 is held on shaft 20 by a screw 21. The peripheral speed of take-off roll 17 is maintained in a predetermined ratio to the speed at which fabric 8 is paid off roll 5 on to plate 14 by means of friction roll 9. With the rate of fabric feed and take-off substantially constant, fabric 8 is under substantially no tension during the operation described. The patterned fabric leaving take-off roll 17 may be allowed to gather and cool on a flat table 22 and is then taken up in any suitable form, such as in roll form, if desired.

To avoid any sticking of the thermoplastic fabric to the heated surface 14, I have found it most advantageous to provide said surface with a suitable heat-resistant lubricant having no undesirable effect on the thermoplastic textile material. The lubricant which yields optimum results comprises a polymeric organic silicone, such as polymeric methyl silicone, the degree of polymerization being such that the polymer has the consistency of a grease.

Any fabric made of or containing yarns or filaments having a basis of a thermoplastic material may be treated in accordance with my novel process. As examples of filament-forming thermoplastic materials of which said yarns may be made, there may be mentioned cellulose esters, such as cellulose acetate, cellulose propionate and cellulose butyrate, mixed esters such as cellulose acetate-propionate and cellulose acetate-butyrate, cellulose ethers, such as ethyl cellulose and benzyl cellulose, synthetic linear polyamide condensation products such as polyhexamethylene adipamide, polymerized vinyl compounds such as polyvinyl chloride, polyvinyl alcohol, polyvinyl acetals, copolymers of vinylidene chloride and vinyl chloride, vinyl chloride and vinyl acetate copolymers and polymerized methacrylic acid compounds. While the most advantageous results are obtained when the fabric is made wholly of thermoplastic yarns and filaments, the fabrics may, of course, also contain a proportion of non-thermoplastic yarns such as those having

a basis of silk, cotton, wool, flax, regenerated cellulose, and the like, woven in any sequence with said thermoplastic yarns.

It is to be understood that the foregoing detailed description is given merely by way of illustration and that many variations may be made therein without departing from the spirit of my invention.

Having described my invention, what I desire to secure by Letters Patent is:

1. Process for the production of patterned fabrics, consisting of the step of passing one side only of an untensioned, undelineated, even-surfaced fabric containing filaments of a thermoplastic material in free, over-all contact with a smooth flat surface maintained at a temperature sufficiently high to effect at least a softening of the thermoplastic material.
2. Process for the production of patterned fabrics, consisting of the step of passing one side only of an untensioned, undelineated, even-surfaced fabric containing filaments of a thermoplastic material having a basis of an organic derivative of cellulose in free, over-all contact with a smooth flat surface maintained at a temperature sufficiently high to effect at least a softening of the thermoplastic material.
3. Process for the production of patterned fabrics, consisting of the step of passing one side only of an untensioned, undelineated, even-surfaced fabric containing filaments of a thermoplastic material having a basis of cellulose acetate in free, over-all contact with a smooth flat surface maintained at a temperature sufficiently high to effect at least a softening of the thermoplastic material.
4. Process for the production of patterned fabrics, consisting of the step of passing one side only of an untensioned, undelineated, even-surfaced fabric containing filaments of a thermoplastic material in free, over-all contact with a smooth flat surface maintained at a temperature sufficiently high to effect at least a softening of the thermoplastic material, said temperature being at least 250° C.
5. Process for the production of patterned fabrics, consisting of the step of passing one side only of an untensioned undelineated, even-surfaced fabric containing filaments of a thermoplastic material having a basis of an organic derivative of cellulose in free, over-all contact with a smooth, flat surface maintained at a temperature sufficiently high to effect at least a softening of the thermoplastic material, said temperature being at least 250° C.
6. Process for the production of patterned fabrics, consisting of the step of passing one side only of an untensioned, undelineated, even-surfaced fabric containing filaments of a thermoplastic material having a basis of cellulose acetate in free, over-all contact with a smooth, flat surface maintained at a temperature sufficiently high to effect at least a softening of the thermoplastic material, said temperature being at least 250° C.
7. Process for the production of patterned fabrics, consisting of the step of passing one side only of an untensioned, undelineated, even-surfaced fabric containing filaments of a thermoplastic material in free, over-all contact with a smooth, flat, lubricated surface maintained at a temperature sufficiently high to effect at least a softening of the thermoplastic material, said temperature being at least 250° C.
8. Process for the production of patterned fabrics, consisting of the step of passing one side

only of an untensioned, undelineated, even-surfaced fabric containing filaments of a thermoplastic material having a basis of an organic derivative of cellulose in free, over-all contact with a smooth, flat, lubricated surface maintained at a temperature sufficiently high to effect at least a softening of the thermoplastic material, said temperature being at least 250° C.

9. Process for the production of patterned fabrics, consisting of the step of passing one side only of an untensioned, undelineated, even-surfaced fabric containing filaments of a thermoplastic material having a basis of cellulose acetate in free, over-all contact with a smooth flat lubricated surface maintained at a temperature sufficiently high to effect at least a softening of the thermoplastic material, said temperature being at least 250° C.

10. Process for the production of patterned fabrics, consisting of the step of passing one side only of an untensioned, undelineated, even-surfaced fabric containing filaments of a thermoplastic material having a basis of cellulose acetate in free, over-all contact with a smooth flat surface lubricated with a polymeric organic silicone and maintained at a temperature sufficiently high to effect at least a softening of the thermoplastic material, said temperature being at least 250° C.

11. Process for the production of patterned

fabrics, consisting of the step of passing one side only of an untensioned, undelineated, even-surfaced fabric containing filaments of a thermoplastic material having a basis of cellulose acetate in free, over-all contact with a smooth flat surface lubricated with a polymeric methyl silicone and maintained at a temperature sufficiently high to effect at least a softening of the thermoplastic material, said temperature being at least 250° C.

FREDERICK G. DODGE.

#### REFERENCES CITED

The following references are of record in the file of this patent:

#### UNITED STATES PATENTS

| Number    | Name           | Date          |
|-----------|----------------|---------------|
| 916,367   | Pohl           | Mar. 23, 1909 |
| 1,889,061 | Dickie et al.  | Nov. 29, 1932 |
| 2,113,935 | Dreyfus et al. | Apr. 12, 1938 |
| 2,120,551 | Dreyfus        | June 14, 1938 |
| 2,199,411 | Lewis          | May 7, 1940   |
| 2,235,869 | Croft          | Mar. 25, 1941 |
| 2,278,896 | Rugeley        | Apr. 7, 1942  |
| 2,284,182 | Verduin        | May 26, 1942  |
| 2,346,208 | Conaway        | Apr. 11, 1944 |
| 2,365,931 | Benger         | Dec. 26, 1944 |
| 2,373,194 | Luttge         | Apr. 10, 1945 |
| 2,373,195 | Wedler         | Apr. 10, 1945 |